

## UNITED STATES PATENT OFFICE

2,516,524

## WHITE CAST IRON

Keith Dwight Millis, Rahway, N. J., assignor to  
The International Nickel Company, Inc., New  
York, N. Y., a corporation of Delaware

No Drawing. Application March 20, 1948,  
Serial No. 16,139

5 Claims. (Cl. 75—123)

1

The present invention relates to white cast irons, and, more particularly, to white cast irons having improved strength especially when produced in the form of sand castings.

It is an object of the present invention to provide a white cast iron having an improved combination of mechanical and physical properties, particularly when produced in the sand cast condition.

It is a further object of the present invention to provide a white iron casting having in the sand cast condition an improved combination of hardness and transverse strength without sacrificing impact properties.

Other objects and advantages of the invention will be made apparent to those skilled in the art from the following description.

Broadly stated, the present invention contemplates a white cast iron composition containing about 2% to about 4.5% carbon, about 0.1% to about 3% silicon, up to about 6% nickel, e. g., 0.01% to 6%, about 0.1% to about 2% manganese, about 0.015% to about 0.5% retained magnesium, up to about 2.5% chromium, e. g., 0.01% to 2.5%, up to about 2% molybdenum, e. g., 0.01% to 2%, and the balance essentially all iron, with exception of small amounts of minor constituents and impurities usually found in cast irons.

It has been found that white cast irons having compositions within the aforementioned range have notably improved strength as compared to similar white cast irons devoid of magnesium. The improved strength of the magnesium-containing white cast irons is reflected particularly in the breaking load determined in the conventional transverse test. The effect of magnesium upon the transverse properties, impact resistance and hardness is illustrated by the following example. A cast iron melt was established containing about 3% carbon, about 0.75% silicon, about 0.2% manganese and about 0.02% sulfur. A portion of the melt was cast without further additions. Two other portions of the same melt were cast after the incorporation of sufficient magnesium to provide retained magnesium contents of 0.04% and 0.06%, respectively, in the final solidified products. The magnesium was introduced as a nickel-magnesium-carbon alloy containing about 11.9% magnesium, 2.8% carbon and the balance essentially all nickel. All three

cast irons were white cast irons in the as-cast condition, as evidenced by the white fracture exhibited by each of the cast irons. The three cast irons had the following properties:

| Percent<br>Mg | Transverse<br>Properties <sup>1</sup> |               | Izod<br>Impact,<br>ft.-lbs. | Brinell<br>Hardness |
|---------------|---------------------------------------|---------------|-----------------------------|---------------------|
|               | Defl.,<br>in.                         | Load,<br>lbs. |                             |                     |
| None          | 0.088                                 | 4,190         | 16                          | 371                 |
| 0.04          | 0.092                                 | 5,380         | 25                          | 375                 |
| 0.06          | 0.111                                 | 6,050         | 28                          | 415                 |

<sup>1</sup> 1.2-inch dia. arbitration bar tested over 12-inch span.

The effect of magnesium in improving the properties, particularly the transverse breaking load, is further illustrated by the following data determined from a white cast iron containing about 3% carbon, about 0.75% silicon, about 0.2% manganese, and about 0.015% sulfur and from a comparable white cast iron which contained, in addition, 0.13% retained magnesium:

| Percent<br>Mg | Transverse Properties |            | Izod Impact,<br>ft.-lbs. |
|---------------|-----------------------|------------|--------------------------|
|               | Defl., in.            | Load, lbs. |                          |
| None          | 0.079                 | 4,580      | 20                       |
| 0.13          | 0.091                 | 5,490      | 27                       |

In order that those skilled in the art may have a better understanding of the invention, the composition and properties of other illustrative white cast irons within the scope of the invention are set forth in Tables I and II, respectively. All the cast irons in these tables were sand cast and were tested in the as-cast condition.

TABLE I

| No. | Per Cent<br>C | Per Cent<br>Si | Per Cent<br>Mn | Per Cent<br>Ni | Per Cent<br>S      | Per Cent<br>Mg |
|-----|---------------|----------------|----------------|----------------|--------------------|----------------|
| 1   | 2.8           | 0.8            | 0.8            | 0.8            | n. d. <sup>1</sup> | 0.024          |
| 2   | 2.8           | 2.1            | 0.8            | 2.0            | 0.012              | 0.064          |
| 3   | 3.4           | 1.8            | 0.8            | 2.0            | 0.016              | 0.061          |
| 4   | 4.1           | 1.3            | 0.5            | 1.8            | 0.02               | 0.06           |

<sup>1</sup> n. d.—not determined.

3  
TABLE II

| No. | Transverse Properties |            | Izod Impact,<br>ft.-lbs. | Brinell<br>Hardness |
|-----|-----------------------|------------|--------------------------|---------------------|
|     | Defl., in.            | Load, lbs. |                          |                     |
| 1.  | 0.070                 | 4,900      | 17                       | 490                 |
| 2.  | 0.104                 | 6,160      | —                        | 444                 |
| 3.  | 0.131                 | 7,250      | 28                       | 375                 |
| 4.  | 0.103                 | 5,870      | 26                       | 418                 |

Many white cast irons containing about 0.75% to 2% nickel, about 2.5% to 3.3% carbon, about 0.5% to 2% silicon and over about 0.04% retained magnesium have been tested and exhibited the following high average properties when tested over a 12-inch span:

Transverse breaking load, 5,600 lbs.

Transverse deflection, 0.102 in.

Within the aforementioned range of compositions, a special range of compositions has been discovered which have particularly outstanding properties which render them especially useful for applications where wear resistance, abrasion resistance and/or high hardness are desired. These compositions contain about 2.5% to 3.3% carbon, about 0.3% to 1.25% silicon, about 3.5% to 5% nickel, about 0.4% to 0.9% manganese, and about 0.05% to 0.1% retained magnesium. The balance of the composition is essentially iron. White cast irons within this special range of compositions have improved properties as compared to similar white cast irons devoid of magnesium but in which some other element, e. g., chromium, is employed as a whitener. The improved properties exhibited by these special white cast irons are particularly notable in sand castings made therefrom. For certain applications, it may be desirable to employ chill castings. White cast irons having the foregoing special compositions will on the average exhibit properties within the following ranges, the transverse load and deflection being determined on 1.2-inch diameter sand cast arbitration bars tested over a 12-inch span:

Load, lbs., 5000 to 6500

Deflection, in., 0.09 to 0.11

Izod impact, ft.-lbs., 20 to 30

Brinell Hardness No. 550 to 715

The aforementioned special white cast irons are characterized by an unusual microstructure not found in other white cast irons having the same nickel content but devoid of magnesium. As is known to those skilled in the art, the microstructure of analogous white cast irons usually will contain massive carbides arranged in a dendritic or cellular pattern. In the special white cast irons of the invention, however, the microstructure is characterized by the presence of carbides in the form of laminations or plates. A notable and unusual feature of the microstructure is the discontinuous nature of the carbide phase. The remainder or continuous portion of the microstructure consists largely of martensite. Tests indicate that the unusual microstructure accounts substantially for the increased strength which has been exhibited by the alloy of the invention.

An unusual characteristic of the aforementioned special martensitic white cast iron of the present invention is that the strength and toughness developed in the sand cast condition are as good or, in many instances, are even better than the strength and toughness developed in

the chill cast condition. In this respect, the magnesium-containing martensitic white cast iron of the invention differs markedly from the analogous magnesium-free white cast irons of the prior art since these prior art white cast irons are generally stronger, tougher and have a higher deflection in the transverse test in the chill cast condition than in the sand cast condition. It has been found that the laminated or plate-like discontinuous carbide structure described hereinbefore and which is characteristic of the magnesium-containing martensitic white cast iron of the invention is particularly well-defined or prominent when the martensitic white cast iron of the invention is sand cast.

The term "white cast iron" is used herein to mean a cast iron (i. e., a eutectiferous alloy of iron and carbon) which has an uncombined or graphitic carbon content not more than about one-half the carbon content in excess of that required to form the matrix, e. g., the eutectoid requirement, and has a white fracture.

In order that those skilled in the art may have a better understanding of the properties exhibited by the special martensitic white cast irons of the present invention, the compositions and properties of martensitic white cast irons within the contemplated range of compositions (Nos. 5, 6 and 7), together with compositions and properties of analogous magnesium-free white cast irons (Nos. 8 and 9), are given in Tables III and IV. All the properties shown in Table III were determined on 1.2-inch diameter arbitration bars cast in sand, except in the case of Nos. 6 and 7 which were chill cast in iron molds. No. 6 had the same composition as No. 5 but differed in that it was chill cast whereas No. 5 was sand cast. All the cast irons were subjected to a transverse test over 12-inch centers after a stress relief treatment for about 3 hours at about 405° F.

TABLE III

| No. | Per cent C | Per cent Si | Per cent S | Per cent Ni | Per cent Mn | Per cent Mg | Others |
|-----|------------|-------------|------------|-------------|-------------|-------------|--------|
| 5.  | 3.3        | 0.4         | 0.009      | 4.5         | 0.4         | 0.07        | —      |
| 6.  | 3.3        | 0.4         | 0.009      | 4.5         | 0.4         | 0.07        | —      |
| 7.  | 3.3        | 0.6         | 0.02       | 4.5         | 0.5         | 0.08        | —      |
| 8.  | 2.9        | 0.7         | 0.1        | 4.7         | 0.5         | none        | 1.5 Cr |
| 9.  | 3.3        | 0.5         | 0.1        | 4.5         | 0.5         | none        | 1.5 Cr |

TABLE IV

| No. | Load  | Defl. | Impact | BHN | Fracture   |
|-----|-------|-------|--------|-----|------------|
| 5.  | 6,380 | 0.003 | —      | 25  | 600 White. |
| 6.  | 5,220 | 0.077 | —      | 23  | 605 Do.    |
| 7.  | 5,850 | 0.089 | —      | 20  | 588 Do.    |
| 8.  | 4,880 | 0.105 | —      | 28  | 511 Do.    |
| 9.  | 4,230 | 0.097 | —      | 26  | 538 Do.    |

Load=Transverse load in pounds applied midway between supports to produce fracture of bar.

Defl.=Deflection in inches at maximum load in transverse test.

Impact=Izod impact value in foot pounds.

BHN=Brinell hardness number.

4.5% Ni-1.5% Cr white iron such as sold under the trade-mark

"Ni-Hard." (Average of 9 heats.)

4.5% Ni-1.5% Cr white iron such as sold under the trade-mark

"Ni-Hard." (Average of 15 heats.)

The martensitic white cast iron of the invention is superior in transverse properties to the ordinary grades of nickel-chromium white cast irons such as are sold under the trademark "Ni-Hard." This superiority is particularly marked in the improved ability of the alloy of the invention to withstand transverse load. It has been found that when tested in the sand cast condition the mar-

tensile white cast irons of the invention can withstand a transverse load approximately 15% to 35% greater than can be withstood by an analogous magnesium-free white cast iron containing about 1.5% of chromium as a whitening agent.

As is known to those skilled in the art, the foundry methods commonly employed to determine the chilling propensity of a given cast iron are the chill block and the step bar. Table V contains the results of tests conducted on chill blocks to show the powerful whitening effect conferred by magnesium in the martensitic white cast iron of the invention. The chill blocks employed had dimensions of 6" x 6" x 2" with the chill being applied on the 6" x 2" face and with the remaining faces of the block being cast against sand. In conducting the tests, the melts employed to produce the chill blocks were superheated to 2850° F. and were cast at 2500° F. The solidified blocks were broken in half in a direction perpendicular to the chill face and were then examined for depth of chill. The results are illustrated by the data in Table V.

TABLE V

Analysis of base iron: 2.8% C, 0.5% Si, 4.5% Ni and 0.35% Mn

| Magnesium content, per cent | White chill, inches | Mottled chill, inches | Gray, inches |
|-----------------------------|---------------------|-----------------------|--------------|
| 0                           | 0.47                | 2.19                  | 3.34         |
| 0.037                       | 0.65                | 2.25                  | 3.10         |
| 0.13                        | 6.0                 | none                  | none         |

A sand cast step bar having the composition of the aforementioned white cast iron containing 0.13% magnesium was completely white in the largest section of a step bar (the two-inch section) after being superheated to a temperature of 2850° F. and being cast at a temperature of 2650° F.

A beneficial effect which has been found to accompany additions of magnesium to the molten cast iron compositions contemplated by the invention is that magnesium has a very powerful desulfurizing effect. It has been found that the reduction in sulfur content which takes place when magnesium is introduced into the molten cast iron consumes a part of the magnesium introduced. Accordingly, when it is desired to introduce the amounts of retained magnesium contemplated by the present invention, it is first necessary to introduce a sufficient amount of magnesium to remove a major part of the sulfur present and to reduce the sulfur content of the white cast iron to a low value. When 0.03% or more retained magnesium is introduced into sulfur-containing cast irons, the sulfur content will be reduced to about 0.02% or even less (e.g., 0.015%). However, if amounts of retained magnesium less than about 0.03% are introduced, the sulfur level in the resulting solidified cast iron may be higher, for example, 0.08%, depending upon the sulfur content of the iron before the introduction of magnesium. The final sulfur will vary inversely with the amount of retained magnesium. In addition to the amount of magnesium required for sulfur removal, a sufficient excess amount of magnesium must be introduced to provide the required retained amounts of magnesium in the final casting. As an empirical approximation, it has been found that of the magnesium actually introduced into the molten cast iron bath

one part by weight of magnesium is consumed for each part by weight of sulfur which is removed from the bath. It has been found that this sulfur-removing property is highly effective regardless of the conditions existing when magnesium is introduced into the cast iron melt. Thus, no slag is necessary in order to carry out the removal of sulfur and the treatment is effective even though the molten metal is held in an acid refractory or is held under acid conditions. Furthermore, no tendency has been found for the sulfur to be re-introduced into the melt when the melt is held after the magnesium treatment. For example, in an instance where 0.096% of magnesium was retained in a cast iron melt containing 3.1% carbon, 0.8% silicon, 4.6% nickel and 0.77% manganese, the sulfur content was reduced from 0.124% to 0.020%. The melt was then held for 20 minutes and, at the end of this time, it was found that the sulfur content was 0.012% and the magnesium content was 0.015%. This loss of magnesium is characteristic of molten magnesium-containing cast irons and is due to a number of factors including oxidation of the magnesium, boiling off of the magnesium as vapor, etc. It can be said that about 0.03% to about 0.06% magnesium is lost in about ten minutes when magnesium-containing molten cast iron is held in hand ladles such as are employed in the foundry.

In all instances where it is attempted to introduce magnesium into molten iron-base baths, it is important to bear in mind the high reactivity of magnesium and to exercise due precaution in order that reactions of explosive violence be avoided. It has been found that if it is attempted to add magnesium to cast iron melts when the melts are at the ordinary casting heat, reactions of explosive violence take place which will propel the molten metal from the receptacle in which it is contained and result in loss of both molten metal and magnesium without introduction of magnesium into the melt. It has been found that metallic magnesium in the amounts contemplated by the present invention could be introduced directly into cast iron melts when the latter are in a pasty condition at a temperature only slightly above the melting point. When this method is employed, it is then advisable after the magnesium introduction to raise the temperature of the bath quickly to a suitable casting temperature in order that sound castings be obtained. A method which has been found satisfactory for the purpose of introducing magnesium into the cast iron melts is to first alloy the magnesium with a metallic composition which is soluble in the molten iron to be treated and in which the magnesium is, in turn, soluble. Satisfactory addition agents are nickel or copper alloys containing up to about 20% of magnesium, e. g., a nickel alloy containing 4% to 20% of magnesium. It is to be pointed out that even in these alloys, the high reactivity of magnesium is still felt. In fact, alloys containing 10% magnesium have been found to burn brightly when placed on top of the molten metal. Recovery of magnesium from the addition agents in terms of magnesium actually retained in the solidified iron casting will vary depending upon the concentration of magnesium in the alloy, the temperature of the bath to which the magnesium is added, the composition of the bath, including the nickel and sulfur contents thereof, etc. Generally speaking, the recoveries of magnesium are rather low; for example, in one instance where

0.5% magnesium was added in the form of a nickel alloy containing 20% of magnesium to a cast iron melt containing 0.05% of sulfur, 0.13% of magnesium was actually recovered in the solidified casting.

The magnesium-containing alloy of the invention possesses an unusual combination of properties, since the transverse strength and deflection thereof are improved above that of analogous magnesium-free alloys without any sacrifice of impact or hardness. Because of this unusual combination of properties, the magnesium-containing white cast iron of the invention finds application in a wide number of fields in which the high hardness, wear resistance, abrasion resistance and moderate toughness of this material may be beneficially employed. For example, grinding balls, attrition mill plates, rolls, pump parts, mining machinery parts, muller tires, nozzles, etc., can be made from the white cast iron of the present invention.

Although the present invention has been described in conjunction with preferred embodiments, it is understood that modifications and variations may be resorted to without departing from the spirit and scope of the invention, as those skilled in the art will readily understand. Variations and modifications apparent to those skilled in the art are considered to be within the purview and scope of the invention and appended claims.

I claim:

1. A casting comprised of a white cast iron containing about 2.5% to 3.3% carbon, about 0.5% to 2% silicon, about 0.75% to 2% nickel, about 0.04% to 0.5% magnesium, less than about 0.020% sulfur and the balance essentially iron.

2. A casting comprised of a white cast iron containing about 2% to 4.5% carbon, about 0.1% to 3% silicon, about 0.1% to about 2% manganese, about 0.01% to 6% nickel, about 0.01% to

2.5% chromium, about 0.01% to about 2% molybdenum, about 0.03% to about 0.5% magnesium, less than about 0.020% sulfur and the balance essentially iron.

5 3. A casting comprised of a white cast iron containing about 2.5% to 3.3% carbon, about 0.3% to 1.25% silicon, about 3.5% to 5% nickel, about 0.4% to 0.9% manganese, not more than about 0.02% sulfur, about 0.05% to 0.1% magnesium, and the balance essentially iron.

10 4. A casting comprised of a white cast iron containing about 2% to 4.5% carbon, about 0.1% to 3% silicon, about 0.1% to 2% manganese, about 0.03% to about 0.5% magnesium, less than about 0.020% sulfur and the balance essentially iron.

15 5. A casting comprised of a white cast iron containing about 2% to 4.5% carbon, about 0.1% to 3% silicon, up to about 6% nickel, about 0.1% to 2% manganese, up to about 2.5% chromium, up to about 2% molybdenum, about 0.03% to 0.5% magnesium, less than about 0.02% sulfur and the balance essentially iron.

KEITH DWIGHT MILLIS.

#### REFERENCES CITED

25 The following references are of record in the file of this patent:

#### UNITED STATES PATENTS

| Number       | Name      | Date          |
|--------------|-----------|---------------|
| 30 1,731,346 | Meehan    | Oct. 15, 1929 |
| 1,874,361    | Rycroft   | Aug. 30, 1932 |
| 2,066,848    | Meuca     | Jan. 5, 1937  |
| 2,145,757    | Ervin     | Jan. 31, 1939 |
| 35 2,336,001 | Eash      | Dec. 7, 1943  |
| 2,370,225    | Boegehold | Feb. 27, 1945 |

#### FOREIGN PATENTS

| Number     | Country       | Date         |
|------------|---------------|--------------|
| 40 360,905 | Great Britain | Nov. 9, 1931 |